

Dec. 12, 1950

P. K. GLASOE ET AL

2,533,452

PHOTOGRAPHIC BRIGHTNESS CORRECTION MASK

Filed June 18, 1947



PAUL K. GLASOE  
DAVID DEAN  
INVENTORS

BY *Newton M. Perina*  
*R. Frank Smith*  
ATTORNEYS

## UNITED STATES PATENT OFFICE

2,533,452

PHOTOGRAPHIC BRIGHTNESS COR-  
RECTION MASKPaul K. Glasoe and David Dean, Rochester, N. Y.,  
assignors to Eastman Kodak Company, Roches-  
ter, N. Y., a corporation of New Jersey

Application June 18, 1947, Serial No. 755,518

7 Claims. (Cl. 95—2)

## 1

This invention relates to photography and more particularly to processes in color photography adapted to producing brightness correction masks of use in printing colored pictures.

In color processes of the type described in Mannes and Godowsky U. S. Patent 2,252,718 granted August 19, 1941, multi-layer color films are described which yield subtractively colored images by means of development with a primary aromatic amino developing agent, the oxidation product of the developing agent combining with the color-forming or coupler compounds to form the dye images. In such processes it has been observed that development in one layer of the color film influences development in an adjacent layer with the effect that exposure in one layer affects density of an image developed in another layer. In these processes the observed effects can be explained on the basis of development that takes place in the black-and-white developer. That is, it is believed that development in a given layer exhausts the developer and releases halogen which slows down development in adjacent layers. The result of these effects, which will hereinafter be called "interlayer effects," is manifest in color pictures produced in processes such as mentioned, as images having varying degrees of brightness, for example, red and magenta images may appear somewhat brighter than other colors in an original color film and when such a film is duplicated in a similar color process the brightness differences are accentuated to the point of being objectionable.

In the corrective processes described in Hanson U. S. Patent 2,294,981 granted September 9, 1942, and Evans U. S. Patent 2,376,132 granted May 15, 1945, are provided colorless silver and colored photographic masks, respectively, which give general corrections for brightness differences in colored images resulting from incorrect absorptions of subtractive dye images. In these processes the use of these types of masks in conjunction with the film to be printed lowers the contrast of the image being printed and requires adjustment of the gamma of the duplicating processes. This adjustment is often very difficult and it would be more convenient if it could be dispensed with. Furthermore, the processes do not provide means for selectively altering the brightnesses of individual colors.

One object of the present invention is to provide means of compensating for said photographic interlayer effects, which results in the rendering of colored images of more uniform brightness in multi-layer color films. Another object of the invention is to provide a masking method which selectively corrects for brightness differences of colored images and particularly of use in duplicating processes. A further object of the invention is to provide a selective masking method which does not appreciably alter the balance of a neutral scale in duplicating

## 2

processes. Other objects will become evident in the following description of the invention.

These objects are accomplished by providing masks which selectively place density back of colors which are too bright when used in conjunction with a color film or transparency in a duplicating process.

The invention may be more readily understood by consideration of the accompanying drawings, wherein,

Fig. 1 shows the conditions which exist in one aspect of the invention in which a subtractively colored film, produced as described in the above patents or by other means yielding subtracting images, in which the interlayer effects have resulted in the cyan scale having a lower gamma in the neutral exposure scale area than in the red and magenta exposure scale areas with the net result shown of obtaining red and magenta colors which are brighter than green and blue colors.

Fig. 2 shows in cross-sectional view, an intermediate stage in forming one of the masks of the invention wherein both silver and dye images are contained in the mask.

Fig. 3 is a cross-sectional view of a corrective mask, made in the manner of the invention, in printing relation to the photographic element of Fig. 1 of which it is a photographic record and which may be used in reproduction processes to correct for variations in brightness of individual colored images.

Fig. 4 shows in cross-sectional view the principal regions of light absorption of the color film of Fig. 1.

In the drawings, Fig. 1 shows the cross-sectional appearance of a reversal processed original color film to be duplicated in the manner of the invention, wherein, layers 1, 2 and 3 contain, respectively, yellow, magenta and cyan dye images in areas of the film corresponding to various exposure scales of the colors indicated across the top of the color film.

By "exposure scale area" or "region" is meant that colored or neutral image-bearing area of a color film which has resulted directly or indirectly from exposure to a range of light intensities of one or more of the primary regions of the visible spectrum. For instance, the "red exposure scale region" is that region of the film of Fig. 1 under R, in which are recorded the range of red light intensities from an original red subject. Similarly, under N in Fig. 1 is shown the record of a range of intensities of white light from an original black-and-white subject.

In Fig. 1, the gamma of cyan in the neutral exposure scale area is shown as being less than the gamma of the cyan in the red and magenta exposure scale regions. This constitutes one aspect of the invention which may be cured by a mask to be subsequently described. The result of the association of these unequal gammas in the film

is to make the reds and magentas appear brighter than the other images of the film because at the same Log. E values, points *a* in Fig. 1, the cyan in the scales of layer 3 has different densities shown as density levels *Nc*, *Mc* and *Rc*. A further result of this condition is evident when the film is duplicated in a similar process. Assuming that the gamma of the cyan in the neutral was 1.0 and the gamma in a red or magenta was 1.2; when the film is duplicated in a process of gamma 1.2 the gamma of the neutral becomes 1.0 but that of the cyan in the red or magenta scales becomes 1.44, thus the condition is accentuated.

In the manner of the invention a panchromatic emulsion layer on a permanent or temporary support is preferably laminated base down onto the color film of Fig. 1. A filtered exposure is made through the color film of Fig. 1 onto the emulsion layer with green light, for example, of wave lengths transmitted by a filter having the characteristics described on page 53 Fig. No. 61 of the publication Wratten Light Filters, seventeenth edition, 1945. This exposure in the upper stratum of the film is developed in an ordinary black-and-white developer of the following composition and washed:

|                                       | Grams/liter |
|---------------------------------------|-------------|
| Na <sub>2</sub> SO <sub>3</sub> ----- | 60          |
| Hydroquinone -----                    | 10          |
| p-Methylamino-phenol sulfate -----    | 2           |
| Na <sub>2</sub> CO <sub>3</sub> ----- | 25          |
| KBr -----                             | 5           |
| NaOH -----                            | 5           |
| NaCNS -----                           | 5           |
| Water to make 1 liter.                |             |

With the masking film in the same printing relation to the color film, a second exposure is made through the color film and the silver image in the masking film with red light such as transmitted by a filter of characteristics described on p. 37 Fig. No. 25 of the above publication. The masking film is then developed in a cyan color developer of the following composition:

|                                       | Grams/liter |
|---------------------------------------|-------------|
| Na <sub>2</sub> SO <sub>3</sub> ----- | 5           |
| 2-amino-5-diethyl amino toluene ----- | 2.8         |
| Na <sub>2</sub> CO <sub>3</sub> ----- | 15          |
| KBr -----                             | 5           |
| p-Methylamino-phenol sulfate -----    | 0.9         |
| NaCNS -----                           | 1           |
| NaOH -----                            | 1.2         |
| Cyan coupler -----                    | 1.1         |
| 6-nitro benimidazole -----            | .05         |
| Water to make 1 liter.                |             |

which may contain one of the cyan couplers disclosed in Vittum U. S. Patent 2,362,598 granted November 14, 1944. As shown in Fig. 2, the film now has silver images and dye images in the strata, but only dye images in areas corresponding to exposures through the magenta and red scales of the film of Fig. 1.

In Fig. 2 of the drawings the photographic element is shown as having a transparent support 4 carrying a panchromatic emulsion layer 5, which for the purposes of describing the invention is divided horizontally into two strata one of which received the first exposure of the invention and in which was developed the silver image; the other part receives the second exposure and contains the subsequently developed dye image. The emulsion layer 5 is further divided vertically into segments corresponding to

the regions of exposure through the exposure scales of the film of Fig. 1.

The printing relation shown in the drawings is that used when the two films are laminated emulsion to base.

The film is then bleached in a ferricyanide-bromide bath and fixed in a hypo solution by conventional means. The result is to obtain a masking film as shown in Fig. 3 wherein the completely processed emulsion layer 3 contains only the cyan masking images 7 in printing relation to the magenta and red exposure scales of the original of Fig. 1. Therefore, it is apparent that when the films of Figs. 1 and 2 are used in registered printing relation when making a reproduction, the images 7 will lower the contrast of the magenta and red exposure scales but have no effect upon the gamma of the neutral scale and the resultant images will be of uniform brightness.

It is apparent that this and the following aspects of the invention may be applied not only to the correction of originals and reproductions produced in the manner of U. S. Patent No. 2,252,718 above identified, but is applicable to any subtractively colored film material requiring these corrections. Also, in forming the final colored images of the invention methods other than color-development, such as toning, may be used for suitably coloring the masking image.

According to a variation of the invention, it is occasionally desirable to place density back of colors other than the reds and magentas. For example, because of faulty exposure, processing, or peculiarities of an original film of the type shown in Fig. 1, it may be required to selectively place yellow back of blue images or magenta behind greens. The condition which exists in such a colored original is similar to that shown in Fig. 1 but when yellow is required back of blues, the gamma of the yellow scale in the blue and cyan exposure scales is higher than that of yellow in the neutral scale. When magenta is required back of the green and yellow exposure scales, the gamma of the magenta in these scales is greater than it is in the neutral exposure scale. Placing yellow back of blue and cyan; and magenta back of green and yellow is accomplished by using suitable wave length of light for the two exposures and processing to the desired colors. To place yellow density back of blue and cyan, the first exposure is made to red light and after silver development the second exposure is to blue light. Following development in the color developer similar to that shown above but containing a yellow coupler, the silver images are removed.

Similarly to place magenta back of greens the first exposure is to blue light and the second to green light. Processing is as previously described using a magenta coupler in the color developer. Suitable yellow and magenta couplers are those such as disclosed in Seymour U. S. Patent 1,969,479 granted August 7, 1934 and Mannes and Godowsky U. S. Patent 2,108,602 granted February 15, 1938.

In most processes utilizing color films of the type described by U. S. Patent 2,252,718 above-mentioned, the density of magenta in a pure red, represented by point *r* on the Log. E axis of the R exposure scale, Fig. 1, is less than it is in the maximum density of the neutral scale, i. e., the magenta dye in the high exposure region of the red exposure scale has a lower density than in the unexposed region of the red exposure scale. Since the amount of magenta in a red is a function of the amount of cyan in a red, as the cyan density in the red decreases, the amount of magenta also

decreases. To correct this deficiency of magenta, it is necessary in making a reproduction to add magenta as a negative function of the cyan in the red and magenta exposure scales only. This is accomplished by making the first exposure as before to green light followed by silver development and after red light exposure through the color film and the silver image, processing in a color developer containing a magenta coupler; or since most processes of this type also require correction for the excessive brightness of the red and magenta colors, the developer may contain both cyan and magenta couplers in suitable proportion or, if desired, a blue-forming coupler such as alpha-naphthol can be used together with the phenylene diamine developing agent.

In another aspect of the invention, which condition may be present in addition to the previously mentioned conditions in a color film, the density of cyan in a green image of a subtractive film may be lower than the density of yellow (see Fig. 1 under G in bottom layer). This may be caused by the overlapping green sensitivity of the red sensitive layer in a multi-layer film of the type described above. Thus, when the green exposure of the original exceeds the threshold value of the red sensitive layer cyan is removed in proportion to the magenta dye formed. The correction required calls for a negative cyan image back of only the green exposure scale of the original being printed. In the manner of the invention this is accomplished by using for the sensitive masking emulsion layer, a panchromatic material of the type described and making the first exposure with magenta (red and blue) light and the second exposure through the color film and silver images with green light. Development between exposures is carried out as before in a black-and-white developer and after the second exposure with a cyan coupler and none or only a minor proportion of magenta coupler in the developer. After removing silver images the result is to place a cyan image in the mask which, when in printing relation to the original, places cyan density back of only green.

In Fig. 4 are shown, in cross-sectional view, the absorption gammas of the dye images in the film of Fig. 1. The areas under the various curves in the yellow, magenta and cyan image-bearing layers 10, 11, and 12, respectively, represent the light absorptions of the various images composing the exposure scales indicated across the top of the film. Thus, the area between curves YB and YG is the blue absorption and the area under YG the green absorption of the yellow dye in the corresponding area of the film of Fig. 1. The areas under the minor absorption curves are colored complementary to the indicated absorption gammas to show that the impure or minor absorptions are effectively equivalent to the presence in minor quantity of another colored material.

The masks made as previously described may be used in combination with a silver brightness correction mask made as described in Hanson U. S. Patent 2,294,981, above, to correct for the impure absorptions of dyes as well as the relative brightness errors of color films. The colored masks of the invention may be combined with a silver brightness correction mask by using as the sensitive masking element a panchromatic silver halide emulsion layer coated on a transparent support over which is coated a black silver filter layer, and over this a red sensitive emulsion layer. The film is laminated base down to the multi-color transparency to be duplicated and exposed

in the manner of the invention with, for example, first green light, then developed to silver, exposed with red light and developed cyan. The silver images are then bleached with a ferricyanide-bromide bath and a third exposure to red light made through the original film. Development is carried out in a low-energy developer compounded as follows:

|    |                                  |       |      |
|----|----------------------------------|-------|------|
| 10 | Sodium sulphite                  | grams | 30   |
|    | Paramethyl amino phenol sulphate | do    | 1    |
|    | Hydroquinone                     | do    | 5    |
|    | Borax                            | do    | 2    |
|    | Potassium bromide                | do    | 0.25 |
| 15 | Water to                         | liter | 1    |

From 50 to 100 mg. per liter of benzotriazole may be added to this developer to inhibit development of the rehalogenized silver. As a result, a silver mask is developed in only the red sensitive emulsion layer since the developer does not develop rehalogenized silver. This leaves a cyan mask over the red colors, and in the top layer a silver mask for correction for the impure absorptions of the dyes of the original and the reproduction processes. If a combined color and tone reproduction mask is desired in the top layer of this film it may be produced therein in the manner of Glasoe U. S. Patent 2,378,213 granted June 12, 1945 by exposing through the highlights of the original transparency with blue light, developing to a high gamma, bleaching with the ferricyanide-bromide bath then exposing with red light and developing in a low gamma developer.

35 In another aspect of the invention, it is not uncommon to encounter in multi-layer subtractively colored films, a condition in which the contrast of the yellow image is lower than the cyan and magenta images. This film or reproduction gives 40 poor pictures, for example, a black object in the original is reproduced with a bluish cast because of the absence of yellow in the higher densities of the neutral scale. This cannot ordinarily be corrected by means of filters, such as yellow, in 45 the reproduction process, because this causes veiling of the highlights with yellow before appreciable correction is obtained in the shadows. This deficiency is compensated for in the manner of the invention by exposing a panchromatic masking film with white light and developing a black-and-white image, the film is then flashed from the emulsion side of the masking film and developed to a yellow positive mask in a color developer containing a yellow coupler. The silver is 50 then removed by conventional means and the film fixed out. The result is a positive mask which when used in printing from the original raises the yellow gamma. The regular red light exposed silver brightness correction mask may also 55 be used in printing with the yellow mask or the two masks may be produced from a single film carrying a panchromatic emulsion layer which is first exposed to red light through the original film, a silver image is then developed, a second 60 exposure is made with blue light and a yellow dye image developed by means of coupler development in the region of the exposure. The previous silver development prevents formation of yellow dye in areas having red transmission. By 65 regulating the amount of blue light exposure, the desired amount of yellow may be added to the blue colors, including the blue areas of the original which should be printed as black or gray.

70 The invention having thus been described, it is 75 to be understood that the disclosure herein is by

way of example, and included in the invention are all modifications and equivalents following within the scope of the appended claims.

What we claim is:

1. The method of forming a brightness correction mask for a photographic color film having colored images composed of subtractive dye images some of said colored images of which appear of different brightness than other colored images and one of said dye images having in a colored image area of said color film a scale of gamma different than the scale of said one dye image in a neutral exposure scale area of said color film, which comprises exposing through said color film a photographic element sensitive to the visible spectrum with light of wave length primarily absorbed by a dye image of said color film common to said colored images of different brightness, forming a silver image in the area of said exposure, subjecting said photographic element to a second exposure through said color film and said silver image with light of wave length transmitted by said brighter images, and forming a colored image in the region of said second exposure of a color substantially the same as said first-mentioned dye image, and thereafter removing said silver image.

2. The method of forming a brightness correction mask for a photographic color film having colored images composed of subtractive dye images some of said colored images of which appear brighter than other colored images and one of said dye images having in a colored image area of said color film a scale of gamma greater than the gamma of said one dye image in a neutral exposure scale area of said color film, which comprises exposing through said color film a photographic element sensitive to the visible spectrum with light of wave length primarily absorbed by a dye image of said color film common to said brighter colored images, forming a silver image in the area of said exposure, subjecting said photographic element to a second exposure through said color film and said silver image with light of wave length transmitted by said brighter images, and forming a colored image in the region of said second exposure of a color substantially the same as said first-mentioned dye image, and thereafter removing said silver image.

3. The method of forming a brightness correction mask for a photographic color film having colored images composed of subtractive dye images of which the red and magenta colored images appear brighter than other colored images and the cyan scale in a colored image area having a gamma greater than the cyan scale in the neutral exposure scale area of said color film, which comprises exposing through said color film a photographic element sensitive to the visible spectrum with green light, forming a silver image in the area of said exposure, subjecting said photographic element to a second exposure through said color film and said silver image with red light and forming a cyan image in the region of said second exposure, and thereafter removing said silver image.

4. The method of forming a brightness correction mask for a photographic color film having colored images composed of subtractive dye images of which the blue colored images appear brighter than other colored images and the yellow scale in a colored image area having a gamma greater than the yellow scale in the neutral exposure scale area of said color film, which comprises exposing through said color film a photo-

graphic element sensitive to the visible spectrum with red light, forming a silver image in the area of said exposure, subjecting said photographic element to a second exposure through said color film and said silver image with blue light and forming a yellow image in the region of said second exposure, and thereafter removing said silver image.

5. The method of forming a brightness correction mask for a photographic color film having colored images composed of subtractive dye images of which the green colored images appear brighter than other colored images and the magenta scale in a colored image area having a gamma greater than the magenta scale in the neutral exposure scale area of said color film, which comprises exposing through said color film a photographic element sensitive to the visible spectrum with blue light, forming a silver image in the area of said exposure, subjecting said photographic element to a second exposure through said color film and said silver image with green light and forming a magenta image in the region of said second exposure, and thereafter removing said silver image.

6. The method of forming a brightness correction mask for a photographic color film having colored images composed of subtractive dye images of which the red and magenta colored images appear brighter than other colored images, the cyan scale in a colored image area having a gamma greater than the cyan scale in the neutral exposure scale area of said color film, the magenta scale in the high exposure region of the red exposure scale having a lower density than in the region of no exposure of the red exposure scale, which comprises exposing through said color film a photographic element sensitive to the visible spectrum with green light, forming a silver image in the area of said exposure, subjecting said photographic element to a second exposure through said color film and said silver image with red light, and forming cyan and magenta images in the region of said second exposure, and thereafter removing said silver image.

7. The method of forming a brightness correction mask for a photographic color film having colored images composed of subtractive dye images of which the red and magenta colored images appear brighter than other colored images, the magenta scale in a colored image area having a gamma greater than the magenta scale in the neutral exposure scale area, the cyan density being less than the yellow density in a green image area, which comprises exposing through said color film with blue and red light, forming a silver image in the area of said exposure, subjecting said photographic element to a second exposure through said color film and said silver image with green light and forming a cyan image in the region of the second exposure, and thereafter removing said silver image.

PAUL K. GLASOE.  
DAVID DEAN.

#### REFERENCES CITED

The following references are of record in the file of this patent:

#### UNITED STATES PATENTS

| Number    | Name           | Date          |
|-----------|----------------|---------------|
| 2,186,053 | Weaver         | Jan. 9, 1940  |
| 2,218,229 | Carroll et al. | Oct. 15, 1940 |
| 2,348,735 | Gaspar         | May 16, 1944  |